

## UNITED STATES PATENT OFFICE

2,142,623

PROCESS FOR THE TREATMENT OF  
TEXTILE MATERIALS

John Rex Whinfield, Manchester, England, assignor to The Calico Printers' Association Limited, Manchester, England, a British company

No Drawing. Application August 17, 1937, Serial No. 159,583. In Great Britain November 8, 1935

1 Claim. (Cl. 91—68)

This invention relates to a process for the treatment of textile yarns, threads, fabrics, fibres, or other materials of cellulosic nature such as cotton and regenerated cellulose rayon, but excluding cellulose esters, with the object of rendering such materials less liable to creasing and to shrinking on washing, and of rendering effects produced by mechanical means on such materials fast to washing.

10 My invention comprises the impregnation of the textile materials with a neutral aqueous solution of a primary water soluble condensation product of urea or a derivative thereof with formaldehyde, drying and conditioning them, subjecting them to a mechanical treatment in order to modify their appearance and thereafter working them in and impregnating them with a cold concentrated acidified solution of a salt having a strong affinity for water but without a specific 15 swelling action on cellulose. By these means any effect produced by a mechanical impress, such as embossed, schreinered or glazed effects, can be rendered fast to washing without the necessity for employing any high temperature heat treatment in order further to polymerize the primary 20 condensation product.

The nature and concentration of the salt solution are such that it exerts little or no swelling action on the material when the latter is immersed therein at room temperature. A suitable salt is calcium chloride and a suitable concentration is 600 gm. litre. Other salts which may be advantageously employed are magnesium and aluminium chlorides. There is room for considerable latitude in respect to concentration and considerable latitude is also allowable as to the time during which the material remains in contact with the saline solution, which may be any period from a few minutes upwards. With the 25 solution just specified, very satisfactory results may be obtained when the period of immersion is about ten minutes. The salt solution contains a small proportion of free acid, for example 1-5 gm. hydrochloric acid per litre, or a somewhat larger quantity of a weaker acid such as acetic acid.

After treating the textile material with the acidified salt solution, the excess of calcium chloride or other salt used is removed by washing first with cold water. After this the material 30 may be soaped at an elevated temperature or given any other suitable washing treatment.

It will be found that by the employment of the above described process the textile material has 35 acquired a satisfactory degree of resistance to

creasing when crumpled, and has become less shrinkable on washing. In the case where the material has been given a mechanical treatment such as embossing after impregnating and drying and before treating in the acidified salt solution it will be found that the mechanically produced effect withstands washing, although this would not be the case if such washing treatment were applied to the cloths before treatment with the acidified salt solution.

10 The above results are achieved without the necessity for a specific treatment of the material at a high or relatively high temperature.

## Example

A viscose rayon fabric is impregnated with an aqueous solution containing 16% by weight of dimethylol urea and 2% of 40% formaldehyde solution. This solution is strictly neutral and contains no catalyst of any kind. It is then dried, 20 conditioned and passed through an embossing calender whereby it receives a figured pattern. Afterwards the cloth is padded in a cold aqueous solution of calcium chloride containing 60 grams of anhydrous calcium chloride in 100 cc. of solution and 1.5% by volume of 28% hydrochloric acid. The cloth thus impregnated is allowed to lie for not less than fifteen minutes, either in folds or wound on a roller, and is then washed first through cold water rendered slightly alkaline 30 with ammonia and finally soaped and dried. As a result of the above treatment, the crease resistance of the material will be found to have been markedly enhanced, and the figured pattern will be found to have been rendered permanent to 35 washing.

The term "conditioning" as employed in this specification is intended to have its ordinary technical significance, namely, as meaning the imparting to textile material of a sufficient moisture content to make it responsive to subsequent operations. Conditioning is essential when the fabric is to be subjected to a mechanical treatment such as calendering, embossing or the like, which would tend to cut the fibre if the latter 40 were not rendered plastic by absorption of a sufficient quantity of water. By "mechanical treatment" is meant an operation such as embossing, schreinering, glazing or the like, mostly carried out on a calender of a suitable type, which imparts to the surface of the fabric a distinctive appearance by the action of pressure, or pressure and friction, and heat.

What I claim is:

A process for the treatment of textile materials 55

of natural or regenerated cellulose which comprises impregnating the textile materials with a neutral aqueous solution of a primary condensation compound of urea or a derivative thereof or with formaldehyde, drying the textile material, conditioning it and subjecting it to a mechanical treatment to modify its appearance, working the

impregnated and mechanically treated material in or impregnating it with a cold, concentrated acidified solution of a salt of the group consisting of calcium chloride, magnesium chloride, and aluminium chloride, and later washing and dry-<sup>5</sup>ing.

JOHN REX WHINFIELD.